# EUROPEAN PATENT SPECIFICATION

(11) **EP 0 114 120 B1**
(45) Date of publication and mention of the grant of the patent: **01.10.1986**
(21) Application number: 84300259.3
(22) Date of filing: 17.01.1984
(51) Int. Cl.: D03D 15/08, D03D 15/00

(54) **Fabric material**
Gewebe
Tissu

(30) Priority: 18.01.1983 GB 8301318
(43) Date of publication of application: 25.07.1984
(73) Proprietor: SCOTT & FYFE LIMITED, Tayport Fife DD6 9DQ Scotland (GB)
(72) Inventor: Tough, William Hamish, Tayport Fife Scotland (GB)
(74) Representative: Hustwitt, Philip Edward

## Description

The present invention relates to fabric material and particularly to woven fabric material including tapes of synthetic resinous material, for example polyamide, polyester, polypropylene, polyethylene.

Tapes of synthetic resinous material and woven fabric materials made from such tapes are stretchable. Methods of forming stretched fabric material including polypropylene tapes are described and claimed in our European Application EP-A-70179 which was filed on 9.7.82 and published on 19.1.83.

The present invention is an alternative and improved method of forming a stretched woven fabric material.

According to the present invention there is provided a method of manufacturing a fabric material comprising the steps of forming a woven base fabric of warp and weft tapes of synthetic resinous material, either the warp or the weft tapes including a series of zones in which the tape is subdivided into a plurality of tapes of lesser width, raising the temperature of the woven fabric, applying tension to the woven fabric to stretch the other of the warp and weft tapes and simultaneously separate the tapes of lesser width in said zones to open gaps of limited length between the said tapes of lesser width, and thereafter cooling the stretched woven fabric in the stretched condition.

The cooled stretched product obtained by the method of the present invention contains gaps of limited length between the said tapes of lesser width. This stretched woven fabric thus has a substantially greater area than the woven base fabric.

It is more convenient to stretch warp tapes of synthetic resinous material in a woven base fabric and it is therefore the weft tapes of the woven base fabric which preferably include the series of zones in which the tape is subdivided into a plurality of tapes of lesser width. These zones are separated from one another by portions of untreated weft tape the presence of which enables the weft tape to retain sufficient transverse rigidity to lie reasonably flat in the woven base fabric.

According to the preferred method of the present invention there is therefore provided a method of manufacturing a fabric material comprising the steps of forming a woven base fabric of warp and weft tapes of synthetic resinous material, the warp tapes being molecularly stretchable in the longitudinal direction and the weft tapes including a series of zones in which the weft tape is subdivided into a plurality of tapes of lesser width, the zones in said series each being separated from one another by an unsplit portion of weft tape, applying heat to raise the temperature of the woven fabric, applying tension to the woven fabric to stretch the warp tapes in the longitudinal direction and simultaneously separate the subdivided weft tapes in said zones to open gaps between the subdivided weft tapes of lesser width, which gaps are limited in length by the unsplit portions of weft tape, and thereafter cooling the stretched woven fabric to obtain a woven fabric of greater area than the originally formed woven base fabric.

The weft tape is advantageously formed with zones in each of which there is a plurality of parallel slits extending longitudinally in the tape with each set of slits in one zone separated from the adjacent similar zone by a portion of flat untreated tape extending substantially perpendicular to the length of the weft tape.

The slits which subdivide each zone in the weft tape are most conveniently formed by pretreating the weft tapes by passing them over the surface of a roller having thereon several rows of pins which penetrate the tape. The roller and the tape are advanced at speeds in a ratio of the order of 1.2 to 1.0 so that the pins form slits of desired length in the tape. Each row of pins thus produces a corresponding row of slits, and the length of the slits is selected such that the row of slits formed by each row of pins is spaced from the succeeding row of slits by an unsplit area or portion of the weft tape. In this portion the weft tape still has its full width.

There is thus obtained an intermittent slitting of the tapes which are subsequently used to form the weft elements in the woven base fabric.

As an alternative to the use of a pinned roller, the slits in the weft tapes can be formed using a roller with interrupted circumferential knife edges, the tape being passed over the roller surface at a speed approximately equal to the roller surface speed.

Conveniently the synthetic resinous material from which the tapes are formed is a polyolefin such as polyethylene or polypropylene.

The present invention will be further understood from the following description of a preferred embodiment thereof which is made by way of example with reference to the accompanying drawings in which :
Figure 1 shows a plan view of a pretreated tape to be used in forming a woven base fabric,
Figure 2 shows a portion of a woven base fabric including tapes similar to the tape of Figure 1 as weft tapes, and
Figure 3 shows the portion of woven base fabric of Figure 2 after being subjected to a stretching treatment.

Referring to Figure 1 there is shown a tape 1 preferably of polypropylene which has therein a series of zones 2 in which the tape has a number of parallel slits 3 causing the tape 1 to be divided, in each of the zones, into several tapes 4 of lesser width.

Each of the zones 2 is separated from the adjacent zone in the series by an unsplit portion 5 which is a portion of tape of the full width of the tape before any slits were formed in it. The unsplit portions 5 of the tape extend transversely of the tape 1 and give the tape transverse rigidity to enable it to remain flat during weaving of the fabric without bunching together of the tapes 4 of lesser width.

The woven base fabric, which is illustrated in Figure 2, is formed using polypropylene tapes 1, i. e. tapes having the zones 2 containing the tapes 4 of lesser width separated by the slits 3, as the weft elements, and untreated polypropylene tapes 6 as the warp elements.

The woven base fabric of Figure 2 is passed through a heating zone, for example in contact with a heated surface, so as to raise the temperature of the fabric to a temperature at which the polypropylene tapes are readily extensible under tension. Advantageously the temperature is a temperature of the order of 160°C at which the polypropylene becomes softened. The woven fabric is tensioned longitudinally of the fabric so that the warp tapes 6 are molecularly stretched to approximately twice their original length. As the warp tapes 6 extend, so the frictional contact between the softened warp and weft tapes causes the subdivided tapes 4 of lesser width in the zones 2 in each weft tape 1 to be separated from one another. Each weft tape 1 thus becomes a series of four smaller tapes 4 united at intervals by the unsplit portions 5, as illustrated in Figure 3.

The unsplit portions 5 may in some circumstances be caused to spread during the stretching of the warp tapes 6. Also the separation from one another of the tapes 4 of lesser width during the stretching of the warp tapes 6 may cause some of the slits 3 to be propagated lengthwise into some of the unsplit portions 5 of the weft tapes 1.

The separation of the four smaller tapes 4 illustrated in Figure 3 is prevented only where an occasional twist occurs in the weft tape 1 as indicated at 8 in that Figure.

The stretched woven fabric shown in Figure 3 is cooled under tension in its stretched condition to obtain a final product corresponding closely in dimensions to the heated stretched woven fabric. The final stretched woven fabric therefore has gaps between the tapes 4 of lesser width.

When stretching of the woven base fabric is effected at temperatures at which the polypropylene becomes softened, bonding occurs between the stretched warp tapes and the various components of the weft tapes at their intersections so that the stretched fabric material is locked and has excellent dimensional stability.

The degree of bonding is controllable by appropriate adjustment of the levels of temperature and tension applied to the fabric, and by the length of time for which the fabric is exposed to the raised temperature.

The stretched fabric material obtained by the method described has approximately twice the area of the original woven base fabric and is composed of warp tapes of approximately half the count of the warp tapes used in forming the original woven base fabric. For example a warp tape 6 of 44 tex used in the original woven base fabric is reduced to approximately 22 tex, and a fabric having warp tapes of such lower count is produced more cheaply by the method of the present invention than it can be produced by weaving an original fabric from warp of that lower count.

The tenacity of the stretched fabric as measured in grammes/dtex is increased as compared with the original woven base fabric.

The stretched woven fabric obtained by the method of this invention has weft tapes with an increased effective width, as compared with the original woven base fabric.

## Claims

1. A method of manufacturing a fabric material comprising the steps of forming a woven base fabric of warp and weft tapes of synthetic resinous material, raising the temperature of the woven fabric, applying tension to the woven fabric to stretch the woven fabric by stretching either the warp tapes of the weft tapes, and thereafter cooling the stretched woven fabric in the stretched condition, characterised in that either the warp tapes or the weft tapes include a series of zones (2) in which the tape (1) is subdivided into a plurality of tapes (4) of lesser width, and in that the tension applied to the woven fabric is applied to stretch the other of the warp and weft tapes and simultaneously separate the tapes (4) of lesser width in said zones (2) to open gaps of limited length between the said tapes (4) of lesser width.

2. A method as claimed in Claim 1, characterised in that the warp tapes (6) are molecularly stretchable in the longitudinal direction and the weft tapes (1) include the said series of zones (2) in which the tape (1) is subdivided into a plurality of tapes (4) of lesser width, and in that the zones (2) in said series are each separated from one another by an unsplit portion (5) of weft tape.

3. A method according to Claim 1 or Claim 2, characterised in that the woven fabric is raised to a temperature at which the synthetic resinous material softens.

4. A method according to any one of the preceding claims, characterised in that there is bonding at the intersections of the warp tapes (6) and the weft tapes (1).

5. A method according to any one of the preceding claims, characterised in that the synthetic resinous material is a polyolefin.

6. A method according to any one of the preceding claims, characterised in that slits (3) are formed in the weft tapes (1) prior to weaving the woven base fabric by passing the tapes over the surface of a pinned roller.

## Patentansprüche

1. Verfahren zum Herstellen eines Gewebes, enthaltend die Schritte : Ausbilden eines Grundgewebes aus Kett- und Schußbändern aus kunstharzmaterial, Erhöhen der Temperatur des Gewebes, Aufbringen von Spannung auf das Gewebe, um das Gewebe zu dehnen, indem entweder die Kettbänder oder die Schußbänder gedehnt werden, und anschließendes Abkühlen des gedehnten Webstoffs in gedehntem Zustand, dadurch gekennzeichnet, daß entweder die kettbänder oder die Schußbänder eine Serie von Bereichen (2) enthalten, in denen das Band (1) in mehrere Bänder (4) geringerer Breite unterleilt ist, und daß die auf den Webstoff aufgebrachte Spannung dazu aufgebracht wird, die Schußbänder bzw. die Kettbänder zu dehnen und gleichzeitig die Bänder (4) geringerer Breite in den genannten Bereichen (2) voneinander zu trennen, um Spalte begrenzter Länge zwischen den genannten Bändern (4) geringerer Breite zu öffnen.

2. Verfahren nach Anspruch 1, dadurch gekennzeichnet, daß die Kettbänder (6) in Längsrichtung molekular dehnbar sind und die Schußbänder (1) die genannte Serie von Bereichen (2) enthalten, in denen das Band (1) in mehrere Bänder (4) geringerer Breite unterteilt wird, und daß die Bereiche (2) in den genannten Serien jeweils voneinander durch einen ungeschlitzten Abschnitt (5) Schußband getrennt sind.

3. Verfahren nach Anspruch 1 oder 2, dadurch gekennzeichnet, daß der Webstoff auf eine Temperatur erwärmt wird, bei der das Kunstharzmaterial erweicht.

4. Verfahren nach einem der vorhergehenden Ansprüche, dadurch gekennzeichnet, daß eine Verklebung an den Überschneidungen der Kettbänder (6) mit den Schußbändern (1) stattfindet.

5. Verfahren nach einem der vorhergehenden Ansprüche, dadurch gekennzeichnet, daß das Kunstharzmaterial ein Polyolefin ist.

6. Verfahren nach einem der vorhergehenden Ansprüche, dadurch gekennzeichnet, daß Schlitze (3) in den Schußbändern (1) vor dem Weben des Grundgewebes durch Leiten der Bänder über die Oberfläche einer mit Stiften versehenen Rolle ausgebildet werden.

## Revendications

1. Procédé de fabrication d'un article textile comprenant les étapes de former un article textile de base tissé ayant des rubans de trame et de chaîne en résine synthétique, élever la température de l'article textile tissé, appliquer une tension à l'article textile tissé pour étirer l'article tissé en étirant soit les rubans de chaîne, soit les rubans de trame, et, ensuite, refroidir l'article textile tissé étiré dans la condition étirée, caractérisé en ce que soit les rubans de chaîne, soit les rubans de trame comportent une série de zones (2) dans lesquelles le ruban (1) est subdivisé en une pluralité de rubans (4) de moindre largeur, et en ce que la tension appliquée à l'article textile tissé est appliquée pour étirer les autres des rubans de chaîne et de trame et en ce que, simultanément, on sépare les rubans (4) de moindre largeur dans lesdites zones (2) pour ouvrir des espaces de longueur limitée entre lesdits rubans (4) de moindre largeur.

2. Procédé selon la revendication 1, caractérisé en ce que les rubans de chaîne (6) ont une structure moléculaire étirable en direction longitudinale et les rubans de trame (1) comportent ladite série de zones (2) dans lesquelles le ruban (1) est subdivisé en une pluralité de rubans (4) de moindre largeur et en ce que les zones (2) dans ladite série sont chacune séparées l'une de l'autre par une portion non fendue (5) de ruban de trame.

3. Procédé selon la revendication 1 ou la revendication 2, caractérisé en ce que l'article textile tissé est porté à une température à laquelle la résine synthétique s'amollit.

4. Procédé selon l'une quelconque des revendications précédentes, caractérisé en ce qu'il se produit une liaison aux intersections des rubans de chaîne (6) et des rubans de trame (1).

5. Procédé selon l'une quelconque des revendications précédentes, caractérisé en ce que la résine synthétique est une polyoléfine.

6. Procédé selon l'une quelconque des revendications précédentes, caractérisé en ce que des fentes (3) sont formées dans les rubans de trame (1) avant le tissage de l'article textile de base tissé en faisant passer les rubans sur la surface d'un rouleau à broches.
